

# UNITED STATES PATENT OFFICE.

WILLIAM HEPWORTH DIXON, OF LONDON, ENGLAND, ASSIGNOR TO THE DIAMOND MATCH COMPANY, OF CHICAGO, ILLINOIS, A CORPORATION OF ILLINOIS.

## MATCH-IGNITION COMPOSITION.

1,341,012.

Specification of Letters Patent.

Patented May 25, 1920.

No Drawing.

Application filed October 11, 1919. Serial No. 330,115.

To all whom it may concern:

Be it known that I, WILLIAM HEPWORTH DIXON, a subject of the King of Great Britain, residing in London, England, have 5 invented certain new and useful Improvements in Match-Ignition Compositions, of which the following is a specification.

The friction surface on a match box is made by applying to the paper label or 10 wrapper a suitable composition, the operation being performed after the label has been pasted on the box.

By this invention a suitable friction composition is applied to the label or wrapper by a printing operation, before the label or wrapper is pasted on the box. This operation may be performed at the same time that the letterpress or the like is printed on the label. For the purpose of the invention the 15 composition is made up as a printing ink or printing color, the active constituent, such as amorphous phosphorus, being incorporated with any suitable known printing composition.

Amorphous phosphorus, however, is not so well adapted as are the usual printing pigments for incorporation with a printing ink composition. I have found, for example, that a composition of sufficient viscosity to be taken up by the main inking roller and containing sufficient amorphous phosphorus, does not leave the printing die readily, thus clogging the machine; it is preferable, therefore, to thin the composition somewhat and to feed it by gravity to the main printing roller. To facilitate this feed the presence of a solid of higher specific gravity than amorphous phosphorus is of advantage; as this weighting material must take the place of some amorphous phosphorus I prefer to use lead peroxid which contributes to the 20 sensitiveness of the striking surface.

The foregoing considerations have led to the following composition as suitable:

Parts by weight.

|                      |     |
|----------------------|-----|
| Copal varnish        | 55  |
| Alumina              | 30  |
| Peroxid of lead      | 105 |
| Amorphous phosphorus | 80  |
| Oil of turpentine    | 50  |

Any of the usual printing ink varnishes may be substituted for copal varnish, which, however, has some advantage in the rapidity with which it dries.

55

The oil of turpentine is the thinning agent, added for the reason stated above; paraffin oil, raw linseed oil or resin oil may be substituted, but they do not dry so quickly.

In making the composition containing 60 lead peroxid care should be taken to dilute the amorphous phosphorus before it is mixed with the peroxid. A safe procedure is thoroughly to mix the amorphous phosphorus with the copal varnish and then to 65 add the peroxid of lead and other ingredients. The final mixture is milled in an ordinary printer's ink mill.

The composition is preferably printed on the paper in the same operation as the printing of the letterpress. For this purpose a 70 separate printing roller placed in the machine either before or after the letterpress printing mechanism, may be used.

Having thus described the nature of the 75 said invention and the best means I know of carrying the same into practical effect, I claim:

1. A match ignition composition comprising a known printing medium having incorporated therewith a material adapted to 80 ignite a match by friction.

2. A match ignition composition comprising a known printing medium and amorphous phosphorus.

85

3. A match ignition composition comprising a printing varnish, a weighting material, amorphous phosphorus and a thinning agent.

4. A match ignition composition comprising a printing varnish, lead peroxid, amorphous phosphorus and a thinning agent.

90

5. A match ignition composition comprising copal varnish, alumina, peroxid of lead, amorphous phosphorus and oil of turpentine in about the proportions specified.

95

In testimony whereof I have signed my name to this specification.

WILLIAM HEPWORTH DIXON.